

Dec. 17, 1929.

C. ELLIS

1,739,581

CONTAINER AND HOOD CAP THEREFOR

Original Filed May 3, 1926

*Fig. 1.*



*Fig. 2.*



*Fig. 3.*



*Fig. 4.*



CARLETON ELLIS  
INVENTOR.

BY *Sol Shappirio*

ATTORNEY.

## UNITED STATES PATENT OFFICE

CARLETON ELLIS, OF MONTCLAIR, NEW JERSEY, ASSIGNOR TO ELLIS-FOSTER COMPANY, A CORPORATION OF NEW JERSEY

## CONTAINER AND HOOD CAP THEREFOR

Application filed May 3, 1928, Serial No. 106,575. Renewed December 31, 1928.

This invention relates to containers and to hood caps therefor, and relates particularly to bottles, the mouth or rim of which is covered and protected by a cap of paper or other fibrous material containing a waxy component of relatively high melting point.

My invention is concerned especially with containers of the milk bottle type such as those having a ledge or seat in the mouth thereof to receive a paper disc, serving as a stopper. Around the mouth of bottles closed in this manner I employ a hood cap, preferably of paper, such hood cap containing plastic material comprising wax of high melting point serving as a binder and stiffening agent. The composition of the hood cap material is such that when heated to a temperature above the melting point of the binder constituents, the paper becomes very plastic and may be pressed around the flange or rim of the bottle, thereby producing a seal which not only keeps out dirt and dust and other contamination, but also provides an indicator, as it were, which shows the consumer whether or not the contents of the bottle have been tampered with in any manner.

In the drawings which are of a conventional diagrammatic character, there is shown by way of illustration, in Figure 1, an elevation partly in section of a milk bottle provided with a hood cap; in Figure 2, a perspective view of a fluted hood cap; in Figure 3, a portion of a bottle having such cap crimped thereon; and in Figure 4, a transverse section through a cap showing portions thereof folded over.

In certain co-pending applications I have specified the employment of carnauba wax, Montan wax, candelilla wax, shellac wax, and similar waxes of high melting point as binders for hood caps, the wax being applied by dipping the shaped cap into a molten mixture of the wax, or spraying the wax in a molten state onto the walls of the cap.

In the present invention I employ emulsions of such high melting waxes as for example, carnauba wax, and I may in one form of the invention introduce such wax emulsion or dispersion into the paper pulp at some stage prior to its formation into a sheet or

web. Thus, for example, the wax emulsion may be added to the pulp in the beater engine.

A second form of the invention involves the spraying of a wax emulsion onto the paper material after it has been sheeted. In some cases, this application of the wax emulsion may be carried out on a part of the sheet, as for example, on one side or a layer of the sheet, as it is being formed in the paper making machine and other layers of paper pulp superposed thereon, giving a finished sheet which has one or more layers of the wax emulsion or dispersion extending throughout the length and breadth of said sheet.

Since, however, a very decided binding and setting action is required to hold the cap firmly in place on the mouth of the bottle, I prefer to use a much larger quantity of wax than would be present if such treatment to form layers of wax only in the interior of the sheet were carried out. Preferably, therefore, I disseminate through the entire mass of the pulp or sheet fine particles of the carnauba wax or other high melting point wax.

When such a substantial proportion of wax is present, the paper when hot is readily moldable and plastic, so that it may be shaped around the mouth of the bottle, and on cooling will harden to form a stiff firm seal or cover, which cannot be dislodged without rupturing sufficiently to indicate tampering, if such has occurred.

A hood cap for milk bottles should contain only substances of a hygienic and sanitary character, free from unpleasant odors and the like. The high melting point waxes aforesaid are satisfactory in this respect. They have other distinct advantages, as for example, they do not stick to the walls of the bottle, but tend to peel from the surface thereof, as I have shown in my co-pending applications. The solidification point is high enough so that the rays of the sun striking on the capped bottle will not render the cap plastic and cause it to spring away from the sides of the bottle.

The emulsion of the wax may be prepared in various ways, as for example, by heating the wax above the melting point with water

and soap and stirring vigorously until the emulsion is secured. A finer and better dispersion is obtained by the employment of the colloid mill, and such finely dispersed wax obtained through this means is especially satisfactory with respect to its dissemination or distribution through the paper pulp, acting as a waterproofing agent, as well as a binder.

10 The use therefore of paraffin wax for waterproofing the hood cap does not become necessary, although a small amount of paraffin wax may be used in some cases to act as a lubricant in drawing the paper through dies to shape into ramekin or cup form.

15 In other cases the carnauba wax in emulsion form, and preferably the milled wax, that is, the highly dispersed wax obtained by means of the colloid mill, may be sprayed onto an absorptive paper sheet after said sheet has been completed on the paper machine. The highly dispersed wax will penetrate quite readily into absorptive paper, waterproofing it and adding a sufficient 20 amount of the high melting point wax to serve as a binding agent when the paper is applied to the mouth of bottles, as aforesaid.

25 By either of these procedures employing the emulsified or dispersed wax I obtain an effect different from that secured by dipping the hood cap into molten wax. The entire texture of the paper is uniform, that is, the wax applied by the emulsion procedure and especially when such emulsion is employed in the 30 beater engine, uniformly distributed or disseminated through the tissue. When such paper material is applied as a cap to the mouth of a bottle and allowed to cool from a plastic to a solid unyielding cover the 35 stresses or strains which are likely to be set up when wax is applied in other ways are not likely to obtain under the present invention, so that a firm capping effect is secured, and moreover, the cap on standing is 40 less likely to loosen slightly and thus rotate about the rim of the bottle.

45 Preferably products tending to loosen slightly in this manner so that rotation is possible, are not desired. The cap preferably should have a very mild adhesion to the walls or rim of the bottle, so that a considerable twist with the hand is necessary in order to loosen the cap. However, the adhesion should not be so great that particles of wax 50 or paper stick to the walls of the bottle in any objectionable degree.

55 Paper sheet made in accordance with the present invention preferably is calendered after leaving the paper machine, such calendering preferably being at a temperature sufficient to soften the wax and render the sheet plastic in order to further enhance the distribution of the wax and compress the milled wax particles into intimate contact 60 with the fibres constituting the paper, and

possibly, in some cases, to actually cause penetration of the wax into the fibre canals.

65 The paper preferably employed in making the hood cap of the present invention is single ply, that is, it is one thickness of paper, made to that thickness on the paper machine (Fourdrinier or cylinder), and is not composed of a series of sheets superposed in order to build up a thicker sheet. Preferably the paper raw material is sulphite pulp, or a mixture of ground wood and sulphite pulp. Usually a proportion of 1 part of ground wood to 3 parts of sulphite pulp is desired, but, in some cases, the proportions may be reversed, that is, 3 parts of ground wood may be used to 1 part of the sulphite pulp. In other cases a mixture of approximately equal parts ground wood and sulphite pulp may be used. The employment of wood pulp, such as that made by the sulphate process, and also the use of other fibrous materials adapted for making sheeted material is within the province of the present invention. In some cases the beating of the stock may be carried out to a rather protracted degree in order to produce a considerable proportion of hydrocellulose, acting as a fixative to hold the wax dispersion in the texture of the paper. In other cases, hydrocellulose separately made may be added in such quantity as is desired.

70 With respect to the paper sprayed with the wax dispersion it is to be expected that the distribution of the wax therein will not be as uniform as that in the case of the paper material made in the beater engine with the addition of the wax dispersion thereto. However, the invention contemplates treatment in both ways in so far as concerns the broad idea of employing an emulsion or dispersion of high melting point wax to yield a paper adapted for hood caps as aforesaid.

75 Other substances such as resins or softer waxes, and the like, may be added to these hard waxes provided such additions do not alter the essential characteristics of said hard waxes. In capping milk bottles it is important that setting takes place rapidly, usually only a few seconds being allowed in which the heated disc or cap is applied to the bottle and must set to a rigid state. The addition of such substances as a considerable proportion of paraffin wax or rosin may cause stickiness, fouling of the bottle, or failure to set with sufficient rapidity. Such additions as are contemplated here are set forth in the main in my co-pending applications aforesaid.

80 Various sizing agents such as rosin size containing free rosin may be employed in conjunction with the high melting point wax dispersion. Such wax may be set with alum or other appropriate setting agent. The carnauba or other hard wax and the rosin size may be used in admixture or they may be 85

introduced into the beater engine separately. For example, the high melting point wax emulsion may be added to the beater engine at the start of the beating operation and at the close rosin size may be added and set with alum and the like. In some cases the wax is first set by adding calcium chloride, aluminum sulphate, or other setting agent and the rosin size then introduced and duly set. The treatment of the paper pulp first with rosin size and afterwards with the high melting point wax dispersion also is not precluded.

The waste or scrap obtained in cutting the discs or sections of the paper which are to be formed into hood caps may be utilized by introducing in small quantities into the beater engine along with fresh paper pulp. In some cases the scrap may be digested with dilute sulphuric or hydrochloric acid to liberate the wax and enable it to be re-emulsified and dispersed. The latter procedure may take place in the presence of the fibre normally in the scrap, or if desired, the wax may be extracted from a part or the whole of such fibrous material.

An emulsion made from 100 parts by weight of carnauba wax, 100 parts of water, 20 parts stearic acid and 2.8 parts caustic soda, all heated to 90° C. and agitated violently, yielded a good emulsion. A mixture of equal parts by weight (dry weight) of sulphite pulp and ground wood, 20 parts altogether, suspended in 400 parts of water was agitated at a temperature of 90° C. with 40 parts of the foregoing wax emulsion. A sheet was formed from this material and this was calendered, first cold and then hot. So large a proportion of wax was introduced in this manner that the sheet was very plastic when hot. However, the fibres of the sheet were so surrounded with wax that the tensile strength was not high. It is proposed therefore to employ proportions of the carnauba wax emulsion of lesser quantity to obtain stronger paper. Thus, instead of 40 parts there may be used 30 parts, 20 parts, or even 10 parts of said emulsion. As the proportion of the emulsion is reduced, rosin size, when used, preferably is increased in amount.

In another case a mixture of equal parts of sulphite pulp and ground wood was emulsified with a dispersion of Montan wax. The sheet formed from this material was calendered at a temperature of 90° C.

In the case of both the carnauba and the Montan wax paper the caps shaped into place on the bottle mouth when the paper was plastic from heating were firmly and effectively attached, moreover, on stripping the paper away from the rim of the bottle, did not leave any matter adhering to the glass.

A milled carnauba wax dispersion may be made as follows:

1/2 gallon of melted carnauba wax and 1 1/2 gallons of a 1 per cent aqueous solution of potassium oleate is introduced into a colloid mill and issues from the mill as a liquid containing the wax in good Brownian movement.

A dispersion is obtained in this manner which has the property of incorporating with fibre effectively and also when sprayed on porous absorptive paper of being readily taken up by the latter, penetrating into the pores of the paper in a notable degree.

Milled carnauba wax or other high-melting point milled waxes thus obtained are regarded as especially desirable in producing a single ply sheet paper material hood cap having an annular skirt. The incorporation in the fibres of the paper of such milled deposited wax yields a non-fouling, quick-setting, hard, high-melting point binder and avoids a coating of wax on the skirt surface, and the invention therefore comprises a bottle container having an enlarged mouth portion in combination with a single ply sheet paper material annular skirted hood cap carrying a non-fouling, hard, high-melting point, quick-setting binder deposited in the fibres of the cap, said cap fitting snugly over the enlarged bottle mouth, with said skirt molded to and under the enlargement of said mouth, the rigidly set contracted portion of the skirt located under said enlargement serving to seal and secure the cap down on the bottle mouth.

An advantage in having the binder deposited or precipitated in the paper instead of, for example, dipping the skirt of the cap in molten binder (carnauba, or other high-melting point waxes) is that wax is not exposed on the surface of the skirt portion when the preferred form of the present invention is utilized. Furthermore, the wax binder in the upper part of the cap (top) assists in overcoming the "spring" of skirt. Stiff paper, bent into cup or ramekin shape when molded against the bottle mouth, will, especially when exposed to a moist atmosphere, tend to open or expand and thus "spring" away from the bottle walls. This may be in part attributed to the difference in water resistance of the top of the cap from the more heavily wax-coated skirt. By having the composition of the paper uniform throughout, as may be accomplished by the present invention, such stresses are much less likely to be in evidence.

The foregoing, however, does not preclude the application to hood caps made in accordance with the preferred form of the present invention, of a coating of wax or other binder, should occasion arise when such dual step is required.

Wax or other high-melting point binder used in this manner may be termed "exter-

nally applied and impregnated". In contrast thereto the deposited or precipitated wax constituting the preferred form of the present invention being substantially uniformly distributed affords a result different from that when the annular skirt of a hood cap is simply dipped in molten wax. Even when the paper material contains a very high proportion of such high-melting point binder, so that when hot and plastic and considerable pressure is applied to the cap on the bottle mouth a small amount of the binder may exude under the pressure applied and coat the paper at the point of such pronounced contact with the glass, it should nevertheless be observed that in the main the bulk of the binder remains in the pores of the paper substantially uniformly distributed, and that, therefore, the springing difficulties observed with hood caps of other types are very little in evidence.

By the term "deposited" as used herein, reference is made to wax which has been thrown down or deposited from a suspension, dispersion, emulsion and the like. This term is used to distinguish over processes wherein the wax is applied by mere dipping of an article into molten wax.

In the drawings A is a milk bottle having a paper disc closure B. C is a paper cap or cup having a desirably smooth top covering the mouth and upper surface of the bottle rim as shown and being bent or crimped around the bottle rim by the pressure of a clamping tool, the groove formed by the latter being shown at D. E is the binding material, while at F such binder is shown as omitted as explained above in connection with one phase of the invention.

40 What I claim is:—

1. A paper hood cap for bottles containing high-melting point, quick-setting wax uniformly deposited in the fibres thereof and serving as a binder to permit the cap to be firmly molded about the mouth of the bottle without employment of externally applied high-melting point wax.

2. In combination with a bottle having an enlarged mouth portion, of a single-ply sheet paper material annular-skirted non-springing hood cap carrying a non-fouling, hard, high-melting point, quick-setting binder comprising deposited wax incorporated in the fibers thereof substantially uniformly throughout the cap; said cap being substantially free from externally-applied and impregnated binder.

3. A skirted paper hood cap containing a wax introduced in emulsified condition with the paper stock in the condition of pulp, the skirt of the cap carrying a binder containing a hard wax and a resin.

4. A skirted paper hood cap containing a wax introduced in emulsified condition with the paper stock in the condition of pulp, the

skirt of the cap carrying a binder containing carnauba wax and resin.

5. A paper hood cap containing a wax uniformly deposited in the fibers thereof in amount sufficient to give a decided binding and setting action.

6. A paper cap made from paper stock containing a considerable proportion of ground wood, said paper carrying a wax deposited in the fibers thereof.

7. A paper cap made from paper stock containing a considerable proportion of hydrocellulose, said paper carrying a hard wax deposited in the fibers thereof.

8. A hood cap made from paper containing a high melting point wax uniformly deposited in the fibers thereof, and set by treatment with a setting agent.

9. A hood cap made from paper containing milled carnauba wax uniformly deposited in the fibers thereof.

10. A container closure shaped by a drawing operation from paper containing a wax uniformly deposited in the fibers thereof, in amount sufficient to give a decided binding and setting action.

11. A container closure shaped by a drawing operation and made of paper having wax introduced thereinto and substantially uniformly incorporated therein.

12. A container closure shaped by a drawing operation and made of paper having incorporated thereinto wax introduced into the paper from an emulsified condition.

13. A container closure shaped by a drawing operation and made of paper carrying a substance acting as a die-lubricant during the drawing operation.

14. A container closure shaped by a drawing operation and made of paper carrying a substance introduced in emulsified condition with the paper stock, said substance acting as a die-lubricant during the drawing operation.

15. A drawn paper container closure containing a hydrocarbon lubricant introduced in an emulsified state into the paper pulp from which the closure is made.

16. A drawn paper product containing a hydrocarbon lubricant introduced in an emulsified condition into the paper pulp from which the closure is made.

CARLETON ELLIS.

120

125

130

70

75

80

85

90

95

100

105

110

115